

1,154,393.

C. W. HILL,  
ELECTRODE FOR ARC LIGHTS,  
APPLICATION FILED AUG. 25, 1911.

Patented Sept. 21, 1915.

FIG. 1



FIG. 3



FIG. 2



FIG. 4



FIG. 6



FIG. 5



FIG. 8



FIG. 9



FIG. 7



Witnesses:

E. B. Gilchrist  
A. J. Hudson

Inventor:

Charles W. Hill  
by Thurston & Davis

Attorneys.

# UNITED STATES PATENT OFFICE.

CHARLES W. HILL, OF LAKewood, OHIO, ASSIGNOR TO NATIONAL CARBON COMPANY  
OF CLEVELAND, OHIO, A CORPORATION OF NEW JERSEY.

## ELECTRODE FOR ARC-LIGHTS.

1,154,393.

Specification of Letters Patent. Patented Sept. 21, 1915.

Application filed August 25, 1911. Serial No. 645,915.

To all whom it may concern:

Be it known that I, CHARLES W. HILL, a citizen of the United States, residing at Lakewood, in the county of Cuyahoga and State of Ohio, have invented a certain new and useful Improvement in Electrodes for Arc-Lights, of which the following is a full, clear, and exact description.

This invention relates to electric arc light carbons and more particularly to those known as flaming arc carbons.

The invention seeks to provide a flaming arc electrode or carbon which while carrying any desired amount of flaming arc material, will nevertheless start upon cold electrode points without assistance or removal of slag.

Generally speaking, the invention comprises elements and combinations thereof set forth in the accompanying claims.

Reference should be had to the accompanying drawings in which—

Figure 1 is an elevation of two electrodes which have been partially consumed. Fig. 2 is a horizontal cross section of one of the electrodes. Figs. 3, 4, 5 and 6 illustrate modifications of the invention. Fig. 7 shows inclined carbons, as distinguished from vertical carbons, as shown in Fig. 1. Figs. 8 and 9 show modifications of the invention.

Flaming arc electrodes as at present made present considerable difficulty and annoyance in their use, because of a scoria or slag which forms as the carbon is burned, which 35 slag accumulates upon the points of the electrodes and forms hard beads or a crust upon the carbon points when the lamp in which the electrodes are employed is out of use. When it is again desired to start the 40 lamp the slag thus formed which is insulating when cold, prevents the electrodes from contacting and thus prevents the formation of the arc. This slag or crust frequently forms when the lamp is burning; 45 that is, the slag forms upon that part of the electrode points which are farthest away from the arc. When, therefore, electrodes feed the slag portions upon the electrodes will contact and prevent the formation of 50 the arc.

It has been proposed to incorporate small amounts of flaming material within the flaming arc electrode which it has been found does not form a slag, but such electrodes when used give an unsteady light of

less intensity than electrodes having a higher percentage of the flaming material, and further, the color of the light given is not satisfactory. Moreover, the degree of inclosure afforded by flaming arc lamps varies considerably in different lamps, and also differs in the same lamp with the removal and replacing of the globe when the lamp is trimmed. Therefore with the present type of electrode it is impossible to prevent the 65 slagging.

In the present invention the electrode is formed of two conducting bodies, one of which is more resistant to consumption in the arc, when used than is the other. Therefore, the less resistant material burns away from the more resistant material, leaving a portion of the more resistant material protruding beyond the end of the carbon. The same phenomena take place upon both the 75 carbons used in a lamp, and therefore when the current is shut off from the lamp, the electrodes will contact with each other upon the protruding portions of the more resistant material. These portions will remain in 80 contact and when the current is again turned on, it will find a ready path through the contacting portions of the electrode, and thus enable the lamp mechanism to properly operate and draw the arc between the electrodes. 85

There are various ways of embodying this invention in practical form, and for purposes of disclosure I have shown a solid carbon A, such as illustrated in Figs. 1 and 2, 90 which is provided with a cylindrical opening extending throughout the length thereof. The body portion A of the carbon itself is composed of carbon mixed with flaming arc material in any proportion which may be desired. Within the cylindrical or cored out portion of the carbon is placed the material B which is more resistant in burning in the arc than is the material forming the body of the carbon proper. This more resistant material may in form assume that of a solid pencil, which is inserted within the opening in the carbon, or if desired, it may be granular material which is mixed 95 with the proper binding material and the same forced into the opening in the carbon.

The material of which the more resistant portion of the electrode is formed, may be any suitable or desirable material, and as instances I would mention petroleum coke, 110

or retort carbon. This material either in pencil form or granular form may be introduced while green into a green carbon, or it may be introduced after the carbon has been baked.

The more resistant portion of the electrode may be allowed to extend beyond the ends of the electrode at the time the electrode is formed, so that in the first instance, there will be projecting portions upon the electrodes within a lamp which may contact even before any burning has taken place. This last construction is desirable, although not necessary. Or the more resistant material may be coextensive in length with the carbon, for as soon as the electrodes are in use, and have burned for a short time, the more resistant material will form a projection C from the electrodes by virtue of the fact that it is not consumed so fast.

While the more resistant material is perhaps preferable in a cylindrical form as indicated in Figs. 1 and 2, this form is not the only form which it may assume, and Figs. 3 to 6 illustrate various modifications which may be employed, Fig. 3 showing an elliptical form; Fig. 4 a star shaped form; Fig. 5 a ring or annulus; and Fig. 6 an electrode having a plurality of more resistant areas.

In Fig. 7 there is illustrated an inclined form of electrode, such as is used upon certain types of lamps. For such use, electrodes would be provided with portions of resistant material which extend along the outer portions of the carbon, as for instance, such as shown in Figs. 8 and 9, the resistant material there being shown as flush with the exterior of the carbon, although it will be apparent that if desired, the same may be in a bead form or extending beyond the sur-

face of the carbon, and extending throughout the length of the carbon. In placing the carbons in a lamp using inclined electrodes, the carbons will be so placed that the more resistant material will be in contact.

Having thus described my invention, I claim:

1. An electrode for flaming arc lamps, having a body portion of flaming material and a good conducting portion of substantially pure carbon more resistant to the action of the arc than is said body portion, whereby the said good conducting portion extends beyond the body portion as the electrode is consumed in the lamp.

2. An electrode for flaming arc lamps, consisting of an outer shell of flaming material and a core of substantially pure, good conducting carbon more resistant to the action of the arc than is said shell, whereby the core extends beyond the shell as the electrode is consumed in the lamp.

3. In a flaming arc lamp, two electrodes for supporting an arc, one of said electrodes having a center of substantially pure, good conducting carbon, and the other having an electrode consisting of an outer shell of flaming material and a central core of substantially pure carbon, said core being more resistant to the action of the arc than said shell, whereby the core contacts with the conducting center of the other electrode when the arc is ruptured and the electrodes are moved together.

In testimony whereof, I hereunto affix my signature in the presence of two witnesses.

CHARLES W. HILL.

Witnesses:

A. J. HUDSON,  
E. B. GILCHRIST.